

## UNITED STATES PATENT OFFICE

FRANZ FÖLGUTER, OF BOCHUM, GERMANY, ASSIGNOR TO THE FIRM DEUTSCHE EDELSTAHLWERKE A.-G., OF BOCHUM, GERMANY

## STEEL ALLOY

No Drawing. Application filed April 5, 1929, Serial No. 352,925; and in Germany May 5, 1928.

Steel alloys are known containing about 1 to 1.5% carbon, 2 to 8% tungsten, 1% chromium and 0.5% vanadium. These steels are used among other purposes for turning 5 grooves in chilled iron mill rolls, a process which is called "riffeling". For this reason these steels are often called rifled steels. They are also used for working in very hard materials such as chilled iron, hard stone, 10 glass or the like, that is, for processes which are carried out at a low cutting speed. In turning chilled iron the cutting speed amounts to 0.7 to 1.0 meter per minute. The work is therefore slow and costly.

15 According to the invention, a great increase in output is attained if the tungsten content is increased to from 10 to 30%, or if, instead of this, an addition of cobalt is made. A very great increase of the cutting output 20 is attained if the tungsten content is increased and cobalt is at the same time added. It has, furthermore, been found that with the above tungsten contents the carbon content can be increased up to 2.5%. In the following table 25 the cutting output of the new steel alloys are compared with the output of those already known. In all cases chilled iron was worked having a "Shore" hardness of 80, the cross-section of the shavings being 2 x 0.5 m/m and 30 the cutting speed 4 m. per minute.

Table

| 35 | Composition |      |     |     |       | Life of tool |
|----|-------------|------|-----|-----|-------|--------------|
|    | C.          | W.O. | Cr. | V.  | Co.   |              |
| 40 | 1.5         | 6.0  | 1.1 | 0.5 | ----- | 7            |
|    | 1.4         | 23   | 1.1 | 0.5 | ----- | 30           |
|    | 1.47        | 6.3  | 1.0 | 0.5 | 10    | 30           |
|    | 1.4         | 22   | 0.7 | 0.5 | 10.4  | 105          |

From this table it will be seen that with steels of the character in question tungsten and cobalt are equal as regards their effect. 45 The considerable increase in the cutting speed

results in economy, owing to the shorter working time and the efficient use of the machines. The alloys described may also be used for purposes in which it is not desired or necessary to take off shavings. In particular they 50 are suitable for drawing dies or matrices subject to severe strain. Their use is suitable for all purposes where extreme hardness and good wearing qualities are necessary. Chromium and vanadium are not absolutely necessary, for obtaining the best values, and other metals such as tungsten, molybdenum and uranium may be added.

The new steels are characterized by exceptional hardness, which is obtained by 60 quenching in oil or water within a wide range of temperatures.

The present steels have nothing in common with known high speed steels. Known high speed steels are used for working on materials with a large area of cut and high cutting speed. The present steel alloy is, however, 65 specially intended for working on very hard materials which necessitate a comparatively small area of cut and a low cutting speed.

Having now particularly described and ascertained the nature of my said invention and in what manner the same is to be performed, I declare that what I claim is:—

1. A cutting steel alloy comprising approximately 10% to 30% of tungsten, approximately from 10 up to and including approximately 10.4% of cobalt, small quantities from a trace to less than 1% of chromium, from 1.4% to less than 2.5% of carbon and the balance substantially all iron, excepting small quantities of impurities and small quantities of other elements commonly present in steels of this type in amounts not greater than 2% in the aggregate.

2. A cutting steel alloy comprising approximately 10% to 30% of tungsten, approximately from 10 up to and including approximately 10.4% of cobalt, small quantities from a trace to less than 1% of chro-

mium, from 1.4% to less than 2.5% of carbon and the balance substantially all iron, excepting small quantities of impurities and approximately 0.5% of vanadium.

5 3. A cutting steel alloy comprising approximately 22% of tungsten, approximately 10.4% of cobalt, approximately 0.7% of chromium, 1.4% of carbon, 0.5% of vanadium and the balance substantially all iron.

10 In testimony whereof I affix my signature.

FRANZ PÖLZGUTER.

15

20

25

30

35

40

45

50

55

60

65